

April 2, 1935.

J. F. WAIT

1,996,181

PROCESS OF FORMING CASTINGS

Filed Nov. 1, 1930

2 Sheets-Sheet 1.

*Fig. 1*



*Fig. 2*



INVENTOR

*Justin F. Wait*

April 2, 1935.

J. F. WAIT

1,996,181

PROCESS OF FORMING CASTINGS

Filed Nov. 1, 1930

2 Sheets-Sheet 2



Fig. 3



Fig. 4



Fig. 5



Fig. 6



Fig. 7

INVENTOR

*Justin F. Wait*

## UNITED STATES PATENT OFFICE

1,996,181

## PROCESS OF FORMING CASTINGS

Justin F. Wait, New York, N. Y.

Application November 1, 1930, Serial No. 492,712

20 Claims. (Cl. 29—148.2)

This invention relates to improvements in methods of constructing such objects as cylinders, vessels and other forms which adapt themselves to fabrication from a metallic alloy. It involves 5 a process of pouring or casting the metal into a shape or form which approximates the ultimate as to general form and in some instances as to size or dimension of substantially all portions of the form.

10 Common procedure for making similar objects involves one of two methods. These are briefly discussed to aid in distinguishing them from the process or method which I have invented.

Castings are generally made from a special 15 composition which is controlled to give high fluidity sufficient to cause the molten metal to flow to all parts of the "imprint" of a shaped mould. This generally is based on the general principle that the melting point of a pure substance 20 is lowered by the addition of another metal which is an "impurity" with reference to the pure metal. It involves the use of special ingredients to lower the melting point and/or to increase fluidity. For example, cast iron is different from steel in 25 composition and bronzes and brasses likewise differ in fluidity from the pure or near pure metals composing the same. A casting is generally made for the purpose of being machined to final dimension and to give smooth surfaces as required. 30 Such castings are considered as being unworkable as by forging.

A second method of construction involves 35 plates, tubing, structural forms and the like which are made by casting an ingot and piercing, drawing, forging or otherwise working the same. The ingot bloom is cast in an unshaped mould which produces a solid mass of metal of appropriate size and shape of outer surface. The composition of the ingot is such as to give the required 40 ductility. On the other hand it is commonly considered that the fluidity of the melt is such that the metal could not be economically poured or cast into forms even approximating that desired as to shape and quality of metal. Metals 45 so worked have special desired properties such as high strength and small grain structure.

50 My invention relates particularly to castings of such alloys as are not adaptable to extensive working as is commonly applied to metals such as iron and soft and mild steel which have, by prior methods, been cast into the well known ingot or bloom which has later been commonly subjected to extensive working and drawing as for example to predetermined length, diameter 55 and wall thickness. On the other hand, such

alloys to which my invention pertains in particular, are possessed of properties which permit of their being worked slightly or somewhat to improve the quality thereof especially as regards rendering them while avoiding appreciable change in shape of the main portion or substantially all thereof. By casting the "unworkable" metal or metal not adaptable to extensive working or metals workable with great difficulty or greater expense, to a form which approximates the ultimate or desired form and working but slightly or materially less than has heretofore been done, the final object may be had in acceptable or improved quality as regards permeability of gases for example and with a great saving in 10 cost of working, wastage and other items inherent to the ingot or bloom manner of forming such objects or ordinary castings which are of poor or less quality than that obtainable by my method. 15

I have found that it is possible to create metals 20 which may be cast into a form approximating for the most part the ultimate or desired form. By form I mean the figure of the object as defined by lines and surfaces. In some instances the size and dimensions of the cast object may be substantially the same as that of the finally desired article. Since the object is cast for the most part to the ultimate figure as defined by lines and surfaces, it is obviously required that most of 25 casting is required to be maintained at approximately the same shape, size and dimension as the casting first formed. If a cylinder is desired, the metal may be poured into a mould and a casting obtained, which approximates the final desired 30 shape. This cylinder may then be worked as by 35 rolling to give the desired grain. The general technique and procedure required to thus perform is known and details are established in accordance with experiment with each alloy and form. This 40 generally improves strength and reduces porosity of such metals which, when cast, have undesired 45 pervious properties especially when operated at a temperature yielding a visible color.

The process of casting generally involves the 50 formation of portions of metal which are of low quality as for example, at the lower and upper regions of a casting. My invention therefore preferably involves the design of a casting in such shape that upper and/or lower portions may be discarded. Porous parts or their equivalent such as portions containing slag are preferably removed so that the remaining portion is substantially homogeneous.

The casting is preferably made of a metal which 55 does not harden or temper at elevated tempera-

tures or which would otherwise act in a manner to reduce the ductility and/or strength at the temperature of working. The metallurgy of alloys suitable for applying my process is known and casting procedure in general is known. A temperature at a near yellow heat or lower is generally satisfactory for working wherefore, the composition is preferably controlled so as to make the metal resistant to oxidation at the working temperature. If the conditions are such that this cannot be conveniently done it is desirable that the working be carried out in a non-oxidizing or in a reducing atmosphere. This may be done as by enclosing the rolls or other working means within a casing or as by excluding substantial amounts of oxygen from a room or chamber in which the piece is worked. If the presence of workmen is required as to control the operation they may be protected as by windows, booths or hoods. An inert gas may be recirculated between the vicinity of the rolls and an outside heat exchange medium to facilitate temperature control.

The working process may involve such steps as rolling, forging and spinning and appropriate combination of such steps. The cylindrical or other form may thus be "drawn", "upset" or otherwise treated at selected points while, as is elsewhere indicated, the main portion of the casting which originally approximated the desired ultimate figure is so held or maintained as to prevent appreciable deviation from the desired form. In producing some objects, the operations may thus include a design alteration, as compared with the desired form such as by enlarging the sectional thickness to furnish the metal required at the selected points. While my invention thus involves casting to the general shape and size, selected portions may be varied as to shape and/or thickness to allow for subsequent change thereof as in the working or for allotting portions which will be caused to contain metal of poor quality and which may then be discarded.

The cast form may be varied somewhat as to shape so as to differ from the final form. For example, if the final section is to be elliptical in shape, a simple and less costly circular form may be cast and the shape varied during the working. It is obvious that where the variation in form is as simple as changing from circle to an ellipse the process is substantially the same and involves no appreciable amount of drawing, forging or similar extensive working. My invention may thus involve steps for altering form such as by cupping, rolling or pressing and with the general limitation that such steps shall not materially lower the quality of the metal as regards the proposed use. Since the main portion of the casting is of the ultimate form or approximately so, such operations are of very limited order except at selected points whereat somewhat more extensive alteration in form may be performed upon portions of the casting preferably particularly made for such working as by enlargement of metal and the like.

The process may be applied to heat resisting metals such as iron containing say about 10% nickel and about 20% chromium and with carbon of say about  $\frac{1}{2}\%$ . Such metals are expensive and difficult to machine. The porosity obtained by casting is undesired for some uses of vessels or other objects made therefrom. Such metal is expensive to weld and the weld is generally of dissimilar composition and otherwise unsatisfac-

tory and is obstinate as regarding working in general.

The above described methods are now usable. A casting may be made. It is porous and requires machining which is quite costly. Many shapes of commercial objects require welding. The method involving ingot production and piercing and/or rolling, etc. is extremely costly because of the vast amount of working that would be required. To do this, at less or reasonable cost, it would probably be necessary to operate at very high temperatures. Many metals oxidize rapidly at temperatures conducive to easy working.

The process may be illustrated as indicated in Figs. 1, 2, 3, 4, 5, 6 and 7. Fig. 1 shows the general procedure used in rolling the casting illustrated as a cylinder. Fig. 2 is representative of a reaction through the rolls and the cylindrical casting being rolled. Fig. 3 shows the shape of the end of the illustrated cylinder after it has been "upset" or enlarged to yield greater thickness of this selected portion of the casting. Fig. 4 shows the "upset" end after it has been worked inwardly by a small amount. Fig. 5 is illustrative of the result of continued inward working of the end. Fig. 6 shows the end after it has been worked to reach the general form of an open dome. Fig. 7 shows the form of the end after the opening of the dome has been closed. It will be noted that the general form of the main body of the casting has been preserved and substantial distortion thereof has been avoided while a selected part, the end, has been appreciably worked.

The roll of Fig. 1 is shown schematically with its fixed frame 1 and removable end 2 carrying driven roll 3, rotating as indicated by the arrow. This roll operates with roll 4 which may be an idler or which may also be driven. The bearings 5 and 6 of roll 4 are capable of causing roll 4 to press against an object 7 being treated. "Set screws" 8 and 9 or power, hydraulic or other "screws" may be used to cause the desired pressure.

A section of the arrangement of rolls is shown in Fig. 2. The exaggerated decrease in thickness of the piece 7 between point 10 and the point of contact with roll 4 is illustrative of the working to produce a better quality and to yield the desired final dimensions. The final shape as indicated by the section between point 10 and roll 4 is thus indicative that the final shape approximates that of the original. Such rolls may coact with other operative parts as required to thus maintain the original shape and form as with particularly obstinate alloys which cannot be subjected to much stress when hot and while being worked to improve grain structure, smooth out irregularities and slightly modify the form to meet the requirements. Such other operative parts may be of known kind or those utilizing known principles of light working.

When treating oxidizable metals or when a gaseous nonoxidizing atmosphere is desired for other purposes as to produce a reducing atmosphere the piece and rolls may be housed to exclude free air. In this manner metal may be treated with a gas. The working effect may facilitate the treatment. Electricity may be passed through the metal as by causing a potential difference between roll 3 and roll 4. Likewise a magnetic or other effect may be used. This or the equivalent is sometimes desirable as while a metal is a conductor in an electric and/or magnetic circuit unusual molecular and/or

crystal conditions exist. These are frequently of value in the treatment especially in combination with working as under the exerted pressure of the rolls.

5 The working of an object less simple in form is illustrated in the third and succeeding figures. A casting may be made of the general shape such as shown in Fig. 3 with appreciable diameter and walls which are relatively thin as regards the 10 diameter. The long body 11 may be worked as by placing the piece on a mandrel carrying a cylinder, either moving or stationary. Outside rolls may be caused to roll relative with the body 11 so as to react with the internal roll in conditions 15 analogous to that of Figs. 1 and 2.

The enlarged lip 12 is what remains after a portion previously existing above has been cut off or otherwise removed. The lips are of greater thickness than that finally desired as they must 20 be enlarged or extended as to surface dimension.

By operating rolls, preferably against a "bucker up" or mould, the lip 12 may be worked as shown in Figs. 4, 5, 6 and 7. The selected portion 12 is shown as relatively small part of the total casting 25 the walls 11 of which comprise the greater portion of the casting. These walls and hence the greater portion of the casting are cast to the exact or approximate final form that is desired. Aside from light working to improve the grain or 30 crystal structure, the major portion of the casting is not appreciably, if at all, altered in form the initial form being retained thus yielding a figure at the end of treatment which is defined by practically or exactly the same lines and surfaces 35 as was the initial casting, except at the selected point 12 which is worked fairly extensively through the stages illustrated by Figs. 4 and 5 and to some stage such as is illustrated by Fig. 6. While in the shape of Fig. 6 a tapered or 40 threaded plug may be inserted into opening 13 and welded tight to yield the form as shown by 14 of Fig. 7. The method renders the amount of machining that is necessary very small or practically negligible. After welding the dome may 45 be rolled or otherwise worked if desired. With some metals other than the chrome nickel metal described, the plug is not always necessary as the hole 13 may be "worked" completely closed. Chrome alloys seem to be difficult to "forge" or 50 work together in a solid manner for such a shape as that described. While the illustration shows inwardly working to form a dome or part thereof, it is to be understood that the working at a selected point need be to effect other change such 55 as that of expanding outwardly or bending over or facing flanges or other parts that may be initially cast. The selected part may also be other than at the end of a cast piece or there may not be a point of appreciable working or there may 60 be a multiplicity thereof and the process may be modified to meet industrial requirements in view of the properties of the alloy.

The aforescribed process thus involves casting of a large portion of the body 11 to approximate shape. The remaining selected portion at 65 12 is worked to a greater extent than that of the body 11. Other methods such as pressing and spinning may be used to work the cast object.

I do not limit my claims to the exact method 70 or procedure as illustrated. Other methods may be used for equivalent purposes, the selection generally depending upon conditions of the metal and the equipment available.

I claim:

75 1. In the process of forming a cylindrical shell

of heat resisting alloy of iron containing nickel, chromium and a smaller amount of carbon and closing one end thereof, the steps which comprise casting into a cylinder approximating the size and shape finally desired, forming an enlarged end, 5 heating to a yellow heat and rolling and spinning the enlarged end to nearly close the end of the cylinder, closing the end, and thereby forming a vessel which is substantially impervious to gaseous fluids. 10

2. The process which comprises casting a heat resisting, stainless steel alloy of iron containing nickel, chromium and carbon into a cylinder approximating that finally desired, heating to a yellow heat, rolling said casting to render it substantially impervious to gaseous fluids and spinning an enlarged end to nearly close the end of cylinder and closing the end. 15

3. In a process of forming a shell with a closed end of heat resisting alloy of iron containing 20 nickel, chromium and carbon the method comprising casting the main body to approximately the desired shape and size, rolling the casting at above a red heat to render the casting substantially impervious to gaseous fluids and simultaneously enlarging the end of the cylinder, 25 working the enlarged end inwardly to approach a closed dome and closing the end forming a closed dome and thereby forming a cylindrical shell and connecting dome which are substantially impervious to gaseous fluid. 30

4. The process of forming a metallic object of selected shape and size of a metal which cannot be worked extensively which comprises casting the object to a size, shape and thickness of metal 35 which is substantially that of the final desired object, removing the portion of the casting containing substantial amounts of slag, working the casting to reduce the porosity thereof while retaining the approximate size and shape of the 40 casting and preventing appreciable change of the main part thereof.

5. The process which comprises forming a casting of metal not adaptable to extensive working said casting being made of the approximate 45 shape and size of a desired object, with a cylindrical body possessed of wall thickness approximating that finally desired, heating to a near yellow heat, working the casting to render the casting substantially impervious to gaseous fluids, and 50 working a selected portion of cylindrical shape inwardly to decrease its diameter appreciably while maintaining the main portion of the cylindrical body at approximately the same shape and size as of the casting first formed. 55

6. The process which comprises forming a casting of metal not adaptable to extensive working said casting being made of the approximate shape and size of a desired object, with a cylindrical body of appreciable diameter and relatively 60 thin walls, heating to a near yellow heat, working the casting to render the casting substantially impervious to gaseous fluids, and working a selected portion of cylindrical shape inwardly to decrease its diameter appreciably while preventing 65 appreciable change in wall thickness of the main portion of the casting first formed, and excluding free air when above a red heat.

7. In forming an object of metal of low ductility by casting the main portion of the body 70 thereof to the desired shape and size of the final product, the method comprising working walls thereof at above about a red heat to reduce the permeability of the walls to gaseous fluid while retaining substantially the same size and shape 75

of the main portion of the body and holding approximately the same wall thickness as of the first cast object.

8. In the process of forming a cylindrical shell 5 of heat resisting alloy of iron containing nickel, chromium and a smaller amount of carbon and closing one end thereof, the steps which comprise forming a cast cylinder approximating the size and shape finally desired, forming an enlarged 10 end, heating to a yellow heat and working the enlarged end so that it will receive a covering piece and applying a covering piece of approximately the same composition and forming a completed dome therewith and so forming a vessel 15 the walls of which are substantially impervious to gaseous fluids.

9. in a process of forming cylinder-like walls 20 of a vessel of heat resisting alloy of iron containing nickel, chromium and carbon which is capable of operating at a red heat and containing gaseous fluid and preventing escapage thereof, the method of casting the object to about the form desired and working the casting at above a red heat to render the casting substantially 25 impervious to gaseous fluid and while preventing appreciable change in the form of the main portion of the casting.

10. The process of forming an impervious cylinder 30 of an alloy which may be worked slightly but not extensively at above a red heat and which alloy is appreciably pervious to gaseous fluid on formation but may be rendered substantially impervious by slight working, which comprises casting the pervious cylinder to a form approximating 35 that desired, working the casting at a near white heat while maintaining its form and so rendering the cylinder substantially impervious.

11. The process which comprises making a casting 40 of a normally gas pervious but resisting alloy in a cylindrical shape in main approximating the desired form of a cylindrical vessel and wherein end is cast in enlarged thickness, working the main cylindrical portion at about a near white heat to render the same substantially impervious 45 while retaining the cast form thereof with practically its initial wall thickness, and working the enlarged end appreciably more than the main body of the casting so as to render it impervious and to shape it that the end of the cylinder may 50 be closed by addition of a separate number.

12. The process which comprises casting an alloy, which may be worked somewhat at a near white heat but which is normally pervious and which is readily oxidized in air at such heat, to 55 a form closely approximating the form of a desired structure, working the casting slightly at a near white heat while excluding air therefrom and imposing a non-oxidizing atmosphere thereon to render the structure impervious and maintaining the casting in approximately the same form 60 during the working and avoiding appreciable distortion of the main body of the casting.

13. The process of forming a structural part of an iron alloy containing about 10% of nickel, 20% 65 of chromium and about ½% of carbon which comprises casting the part to approximately the form desired, working the metal a little at about or near white heat to render it substantially impervious as regards gaseous fluid at high temperatures of application of the metal and maintaining approximately the same cast form and 70 thickness throughout the working.

14. The process of claim 13 wherein a selected point of the casting is made heavy and worked appreciably in excess of the main body and with appreciable change in form of the selected point.

15. For the purpose of treating a casting of an alloy which is particularly obstinate as regards working and effectively working it to improve its grain structure and avoiding the necessity of extensively working the same to attain a cylindrical form, the method of casting the cylindrical form 10 to the approximate diameter and wall thickness as finally desired, and working the casting at above a red heat and below a white heat while preventing appreciable alteration in diameter and wall thickness.

16. The process of improving a cylindrical casting of heat resisting alloy while avoiding substantial change in size and shape of the main portion thereof which comprises casting the alloy to about the desired form and size and subsequently working the casting at about a near yellow heat in a manner largely to improve the grain structure and render the metal practically impervious to gaseous fluid and while avoiding substantial 20 change in the size and thickness of the main 25 portion of the casting.

17. The process of forming a metallic object of substantial diameter and relatively thin walls while avoiding extensive working of the main portion thereof which comprises casting the object 30 in approximately cylindrical form to a size and of a shape about as desired and working the casting at high temperature to decrease the pore size while preventing appreciable change in the form and the size and thickness of the main 35 portion of the casting and so producing an improved object with but little change in size and of about the same thickness of metal as regards the main portion of the original casting.

18. The process of improving a casting of heat 40 resisting alloy by small working at elevated temperature which comprises casting the object so that the main portion of the casting conforms fairly closely with the size, shape and thickness 45 of that of the desired structure, working the casting at substantially elevated temperature to remove most of the permeability to gaseous fluid inherent to the casting and while maintaining its approximate form and avoiding substantial distortion of the main portion of the casting.

19. The process of forming an object of selected 55 shape and size of a metallic alloy which is obstinate as regards working and cannot be extensively worked and is normally porous which comprises casting the object to substantially the desired metal thickness, size and shape and working the casting to improve the grain structure and reduce the porosity while avoiding material change in form, size and thickness of the main 60 part of the casting.

20. In forming a metallic object of a metal which cannot be extensively worked but which may be worked by a small amount, the steps comprising casting the object to a form approximating that desired and removing portions of 65 undesired metal and working the casting to improve the grain structure and reduce inherent porosity of the casting while retaining the approximate size and shape of the casting and avoiding material distortion of the main part 70 thereof.

JUSTIN F. WAIT.